

1

3,446,736  
**MIXED CARBOXYLATE DERIVATIVES OF BASIC  
ALKALINE EARTH METAL SULFONATES**  
Richard S. Herd and Ferdinand P. Otto, Woodbury, N.J.,  
assignors to Mobil Oil Corporation, a corporation of  
New York  
No Drawing. Filed Feb. 8, 1968, Ser. No. 703,868  
Int. Cl. C10m 3/34  
U.S. Cl. 252—33.2

16 Claims

## ABSTRACT OF THE DISCLOSURE

Overbased, carbonated alkaline earth metal sulfonates, having a metal content at least 200% higher than that of a corresponding normal metal sulfonate salt, are reacted with formic acid and a second carboxylic acid containing from 2 to about 5 carbon atoms to provide improved oil-soluble detergents for lubricants and as an additive for fuels. The process for preparing these oil soluble salts requires at least two steps in which the formic acid is reacted with the said sulfonate first followed by the reaction with the second carboxylic acid. The ratio of chemical equivalents of acids ranges from about 40:1 to 1:4 of formic acid to the second carboxylic acid.

## BACKGROUND OF THE INVENTION

### Field of the invention

This invention relates to oil soluble, overbased alkaline earth metal sulfonate derivatives and to methods for preparing the same, and in particular, it relates to mixed carboxylate derivatives of the sulfonates.

### Description of the prior art

U.S. Patent No. 2,763,615 deals with the reaction product of a low molecular weight monocarboxylic acid with a barium salt of a sulfonic acid. However, this reference only discloses low-metal containing salts. U.S. Patent No. 3,027,325 discloses preparing a mixture of calcium sulfonate, calcium hydroxide, water and alcohol in an oil and reacting with carbon dioxide. There is no disclosure in this reference of reaction with an acid.

## SUMMARY OF THE INVENTION

It has now been discovered that alkaline earth metal carbonate-sulfonate salts may be reacted with formic acid and a second carboxylic acid having from 2 to 5 carbon atoms whereby the metal carbonate portion of the salt is converted to the formate-carboxylate to produce liquid, oil-soluble products which possess improved characteristics in lubricating oil. The ratio of formic acid to the C<sub>2</sub> to C<sub>5</sub> acid may range from about 40:1 to 1:4, and preferably from 10:1 to 1:3.

## DESCRIPTION OF SPECIFIC EMBODIMENTS

It has been found that the reaction of metal carbonate-metal sulfonate salts, as they are also referred to herein, with acetic acid or higher acids result in the formation of gel-like, oil-insoluble masses. As such, they would be unsuitable for use as a fluid lubricant. On the other hand, the reaction of these carbonate-sulfonate salts with formic acid alone, in the presence of a diluent, preferably an oil diluent, produce excellent, liquid oil-soluble detergents and corrosion inhibiting additives. The basicity of the salts is high enough to prevent the corrosion caused by acids derived from oxidation of the oil or combustion of sulfur containing fuels. Occasionally, however, the water stability of such formic acid derivatives, while satisfactory, is not always optimum. It is, therefore, surprising to discover

that by converting the carbonate portion of the sulfonate salts to the formate initially and then converting the remaining portion of the carbonate to a higher carboxylate, until substantially all of the carbonate has been converted, the resulting salts remain liquid and oil soluble. The basicity is retained at the level required to help prevent corrosion of metal surfaces in the engine and the water stability is considerably improved. If desired, some of the metal carbonate may still be permitted to remain in the reaction product. Complete conversion of the carbonate is not essential.

For the sake of simplicity, the products of the present invention and the overbased metal sulfonates from which they are obtained will hereinafter be referred to using terminology such as metal sulfonate-metal carbonate or metal carbonate-overbased metal sulfonate for the intermediate product and metal sulfonate-metal carboxylate or metal carboxylate-overbased metal sulfonate for the final product, or similar expressions. The precise structure of the metal carboxylate-containing products of the instant invention is not known. Without limiting the invention to any particular theory, it is believed that the several components form a product of the dispersion or colloidal suspension type wherein the mixed metal carboxylates are held in dispersion or suspension by the metal sulfonate.

A variety of overbased, metal sulfonate-metal carbonate salts, which are suitable for use in the mixed carboxylic acid reaction of the present invention, are shown in the art. Typical of these and, indeed, preferred, are the metal carbonate-overbased metal sulfonates described in U.S. Patent Nos. 2,616,911 and 2,956,018.

As disclosed in U.S. in U.S. Patent No. 2,956,018, these metal carbonate-overbased, metal sulfonates may be prepared by admixing an inorganic compound of a basic metal, such as an alkaline earth metal oxide or hydroxide with an aliphatic monohydric alcohol containing 1 to 5 carbons such as methanol. A metal carbonate reagent is then formed by passing carbon dioxide through this admixture of the basic metal compound and the aliphatic alcohol. This metal carbonate reagent is reacted with a sulfonic acid or sulfonic acid salt to form the metal carbonate-overbased metal sulfonate, which is reacted with the carboxylic acids according to the present invention.

In view of the fact that calcium sulfonate-calcium carbonates are of special interest, the following is a further more specific description of one of the preferred methods of preparing a calcium sulfonate-calcium carbonate which may be used in the preparation of the high metal content overbased, metal sulfonates of the present invention.

The formation of the calcium sulfonate-calcium carbonate involves the preparation of a calcium carbonate reagent in methanol and the reaction of this reagent with a sulfonic acid or sulfonate salt. The resulting calcium sulfonate-calcium carbonate is then reacted with formic acid and a second acid to form our metal mixed-carboxylate products.

More particularly, the aforementioned calcium carbonate reagent may be prepared by carbonating with carbon dioxide a suitable calcium inorganic compound such as calcium oxide or hydroxide in methanol. For example, the reagent may be prepared by first forming a suspension of the calcium compound, e.g., calcium hydroxide in absolute methanol, adjusting the temperature of this suspension to below approximately 30° C., preferably so that amount of carbon dioxide absorbed is such as to provide a mol ration of carbon dioxide to calcium therein of from about 0.6 to about 2.0.

The resulting calcium carbonate reagent is then reacted with a suitable sulfonic acid or metal salt thereof as follows. The chilled (10–30° C.) reagent is intermixed with a solution of the sulfonic acid or salt in mineral oil

and the mixture is heated to a temperature above the boiling point of methanol to facilitate reaction and effect removal of the methanol by distillation. After the distillation step, the reaction mixture is filtered, preferably while hot, to provide the high metal-content calcium sulfonate-calcium carbonate.

A sufficient amount of mineral oil is preferably employed as solvent in the reaction between the calcium carbonate reagent and the sulfonic acid or salt in order to maintain the reaction mixture fluid and thus facilitate the final filtration and handling of the product which would otherwise be quite viscous. Other hydrocarbon solvents besides mineral oil or in addition to mineral oil, such as light naphtha, xylene, toluene, benzene, etc., may be employed.

The amount of calcium carbonate reagent employed in the reaction with the sulfonic acid or salt should, of course, be sufficient to provide the excess metal which is incorporated into the salt product. Thus, at least about 3 equivalents and up to about 31 equivalents or more of calcium should be provided in the reagent where the sulfonic acid per se (i.e., unneutralized) is used and at least about 2 equivalents and up to about 30 or more of calcium, where a neutral sulfonic acid salt is utilized in the process, the said equivalents being on the basis of the acid-hydrogen equivalents of the sulfonic acid or the neutral sulfonic acid salt.

Other methods of preparing carbonated, basic alkaline earth metal salts may be used, such as simply reacting an alkaline earth metal oxide or hydroxide with a sulfonic acid or normal sulfonate salts in the presence of a lower aliphatic alcohol, such as methanol, and passing carbon dioxide therethrough.

The sulfonic acids from which the calcium sulfonate-calcium carbonate intermediates are prepared, or, indeed, any of the metal sulfonate-metal carbonates, include oil-soluble petroleum and synthetic alkaryl sulfonic acids, particularly those having molecular weights of from about 300 to about 1500. These acids may be produced by sulfonation of petroleum stocks or synthetic alkyl aromatic compounds, such as alkyl substituted benzenes and naphthalenes, wherein the alkyl groups attached to the aromatic ring contain at least about 12 carbon atoms and preferably from at least about 14 to about 24 or more, carbon atoms. Suitable synthetic sulfonic acids are, for example, octadecyl-benzene sulfonic acid. Of the various acids, the wax benzene and wax-naphthalene sulfonic acids and mixed alkyl aromatic sulfonic acids are preferred. The petroleum sulfonic acids, also known as "sour oils," are those obtained in the treatment of petroleum oils, particularly refined or semi-refined oil, with concentrated or fuming sulfuric acid, and which remain in the oil after settling out of sludge. These sulfonic acids may be represented by the general formula:



where R is one or more alkyl, alkaryl or aralkyl groups and the aromatic nucleus is a single or condensed ring or partially hydrogenated ring. Other suitable sulfonic acids, such as aliphatic sulfonic acids, derived from polyolefins having a molecular weight of from 300 to 1500, paraffin wax, and the like, may be used in this invention.

Although the preparation of the calcium carbonate-overbased, calcium sulfonate intermediate has been referred to in some detail, it should be noted that the present invention is applicable to any overbased, metal sulfonate containing a metal carbonate as the overbase material wherein the metal is an alkaline earth metal. It will also be appreciated that any of this type of metal carbonate-overbased, metal sulfonate products may be employed in the formic acid-C<sub>2</sub> to C<sub>5</sub> acid reaction regardless of their particular method of preparation.

Overbased metal sulfonate-metal carbonate compositions wherein the metal used is an alkaline earth metal,

preferably calcium, barium, or strontium, are reacted initially with formic acid followed by the reaction with the higher carboxylic acid. The total equivalents of acid added to the reaction mixture is preferably sufficient to at least substantially convert all of the basic carbonate to the mixed carboxylate. There is thus approximately one total equivalent of the acids per equivalent of carbonate employed in producing the products of this invention. The reaction with the acids is conducted at slightly elevated temperatures to high temperatures. Temperatures in the range of from about 50° to about 225° C., preferably from about 100° to 200° C., are suitable. If a diluent for the reaction mixture is used, it is preferably a refined mineral oil and may constitute from 20% to 80% of the reaction mixture.

The reaction product may be recovered in any suitable manner, such as by filtration, wherein the desired reaction product is recovered as the filtrate. Satisfactory filtration results are obtained by adding a small amount of a sulfonic acid to either the formic acid or the C<sub>2</sub> to C<sub>5</sub> acid or both used in the reaction step. Any sulfonic acid may be mixed with the carboxylic acid. For example, sulfonic acids, such as those hereinabove mentioned as suitable for use in the preparation of the metal sulfonate-metal carbonate products may be employed. The rate of filtration may be further improved if the reactions between the carboxylic acids and the metal sulfonate-metal carbonate are conducted at temperatures from about 100° to about 200° C.

The criticality of reacting the metal carbonate-overbased metal sulfonate with formic acid first is demonstrated by the fact that corresponding metal acetate-overbased metal sulfonates are gel-like, insoluble masses unsuitable for use in producing fluid lubricating oils. Reaction of the sulfonate-carbonate with formic acid as the first step, followed by reaction with the C<sub>2</sub> to C<sub>5</sub> acid prevents gelation of the reaction product. If desired, the acid reaction may be performed in a series of 2, 3, 4, or more steps providing always that the first step involves reacting formic acid alone. Formic acid must not be pre-mixed with the higher acid in the initial step. Hence, in the first step, formic acid is reacted with a portion of the carbonate component. The second step consists of reacting with acetic acid or higher molecular weight acid. If desired, the first two steps may convert only a portion of the carbonate. A third step may consist of reacting more formic acid or even a third acid with the remainder of the carbonate or this step may in turn be followed by a fourth reaction with a higher acid, providing the ratio of acid equivalents is met. Mixtures of C<sub>2</sub> to C<sub>5</sub> acids may, of course, be used.

The C<sub>2</sub> to C<sub>5</sub> acids consist of acetic acid, propionic acid, butyric acid and valeric acid or the anhydrides thereof, and branched isomers as well. As much as 4 to 1 of the higher acids to formic acid may be employed, however, higher mole ratios result in gelation.

The metal mixed carboxylate-overbased metal sulfonates of this invention possess additive properties superior to those of the corresponding metal carbonate-overbased metal sulfonates. Thus, our metal carboxylate products inhibit the deposit-forming tendencies, increase the high temperature stability and improve the anti-wear properties of lubricating oils to a significantly greater extent than do the corresponding metal carbonate products.

The metal carboxylate-overbased metal sulfonate products of this invention are further distinguishable from metal sulfonate products heretofore known, by virtue of their remaining liquid even with exceedingly high metal contents. Thus, the metal contents of our metal carboxylate overbased products are from 200 percent up to about 2000 percent or more, higher than that of the corresponding "normal" salts, i.e. salts having metal contents equivalent to the acid hydrogen contents having the respective sulfonic acids from which they are derived.

The production of metal carboxylate-overbased metal sulfonates containing such high metal contents is due to

the specific procedure utilized in our synthesis. According to this aspect of the invention, the metal carboxylate-metal sulfonate product is produced by going through the carbonate group of the metal carbonate-overbased metal sulfonate, that is, by first forming the metal carbonate-overbased metal sulfonate and then converting this product to a metal mixed carboxylate-overbased product by reaction with formic acid followed by the  $C_2$  to  $C_5$  acid. The importance of this specific process procedure becomes apparent when it is realized that metal sulfonate-metal carboxylate products, such as calcium sulfonate-calcium carboxylate products, possessing metal contents from 200 percent up to 2000 percent or more higher than that of the corresponding normal salt, as far as we are aware, cannot be prepared directly from a sulfonic acid or calcium sulfonate and a carboxylate. According to the best of our knowledge, only by carrying out the instant formic acid reaction initially is it possible to produce such extremely high metal content calcium sulfonate-calcium carboxylate oil-soluble products, since there is believed to be no other effective way of introducing such amounts of calcium carboxylate other than by going through the carbonate group.

These metal sulfonate-metal carboxylate products are of particular interest as additives for marine diesel cylinder lubricants wherein they inhibit the deposit-forming tendencies especially the port clogging tendencies which result from the use of high sulfur content fuels in these engines, and act to improve the anti-wear characteristics of the lubricating oils. These metal carboxylate overbased products may also be used, for example, in lubricating oils for railroad diesel engines, gas engines, as well as in as various other types of lubricants for internal combustion engines. It will be appreciated, however, that the products of the present invention may be advantageously used in a variety of mineral oil lubricating compositions. The products may also be used in gasoline and fuel oil for de-  
20 tergency or other utility, i.e. reduction of corrosion.

The particular amounts of the metal carboxylate-overbased sulfonate product used in the final fluid compositions will depend on factors such as the nature of the base stock, its intended use, the presence of other ingredients, etc. In general, the overbased sulfonate product may be present in an amount from about 0.05 to 50 percent by weight of the base, or higher, if desired. In the case of marine diesel oils higher proportions in the range of from about 20 to 40 percent, preferably 25 to 35 percent are used. On the other hand, in automotive engine oils, 0.5 to 20 percent, preferably 1 to 10 percent of the additive may be used.

It will of course, be appreciated that the mineral oil compositions containing the instant overbased sulfonate product may, of course, also contain effective quantities of various other typical lubricating oil additives, such as pour point depressants, V.I. improvers, extreme pressure agents, anti-oxidants, etc.

The following examples are presented to illustrate more clearly the nature of the present invention. It should be understood, however, that the invention is not limited to these specific embodiments.

Example 1 shows the procedure for the preparation of a calcium sulfonate-calcium carbonate product which is of the type reacted with formic acid and the  $C_2$  to  $C_5$  acid in the succeeding working examples.

#### EXAMPLE 1

A slurry of 148 grams (4.0 true equivalents) of calcium hydroxide in two liters of absolute methanol was charged into a 5-liter flask, chilled below 15° C. in an ice-bath and carbonated to a carbon dioxide:calcium ratio of 1.9 (162 grams, 7.4 equivalents of  $CO_2$ ). The slurry thickened considerably during the carbonation. The rate of carbonation was followed by noting the increase in weight of the reaction flask.

A mixture of 600 grams (0.67 true equivalents) of a mixed wax-benzene (2-12)-alkyl aromatic sulfonic acid

having a total N.N. of 68 and a true N.N. of 63 and 600 grams of diluent oil (a paraffinic oil having a viscosity of 100 SUS at 100° F.) was heated in a beaker to 60° C. and added to the carbonated reagent.

5 The methanol was removed through a Dean-Stark take-off by heating the reaction mixture to 90° C. over 6 1/4 hours and then maintaining the temperature at 90-100° C. for 1 1/2 hours with vigorous nitrogen blowing.

10 Sixty grams of "Hyflo" (a diatomaceous earth filter aid) was added and the mixture filtered through an electrically heated Buchner funnel precoated with "Hyflo" giving a bright fluid product having the following analysis:

15 Total calcium, percent ----- 5.3.  
Perchloric acid base No. (mg.  
KOH/g. sample) ----- 120-4.3% calcium.  
Excess calcium, percent ----- 430.

#### EXAMPLE 2

20 One-hundred grams (0.214 equivalents of  $CO_2$ ) of a calcium sulfonate-calcium carbonate product (4.7%  $CO_2$ , 5.1% Ca., 121 TBN, prepared according to Example 1) were charged into a 250 ml., 4-neck round-bottom flask equipped with a mechanically driven glass paddle type stirrer and a thermometer. The charge was heated to 90° C. and 5.0 grams (0.098 equivalents) of 90.5% formic acid were added slowly above surface dropwise. After the formic acid addition, the reaction mixture in the flask was heated to 120° C. and 5.1 grams (0.089 equivalents) of 97.4% acetic anhydride was added dropwise. During the acetic anhydride addition, 50 grams of a solvent refined mineral oil diluent was also added. The reaction product was then heated at 150° C. with a stream of nitrogen for one hour, and 7.5 grams of diatomaceous filter aid was added to the mixture. The mixture was filtered through diatomaceous filter aid on a heated Buchner funnel. The resulting product was a liquid.

#### Analysis of product:

|                                              |         |      |
|----------------------------------------------|---------|------|
| Calcium                                      | percent | 3.1  |
| Carbon dioxide                               | do      | 0.91 |
| Formic acid <sup>1</sup>                     | do      | 1.8  |
| Acetic acid <sup>1</sup>                     | do      | 2.9  |
| Perchloric acid base No. (mg. KOH/g. sample) | 74      |      |

40 1 As formate and acetate of calcium.

#### EXAMPLE 3

45 To 500 grams (1.07 equivalents of  $CO_2$ ) of a calcium sulfonate-calcium carbonate product similar to that used in Example 2 was added a mixture of 25 grams (0.49 equivalents) of 90.5% formic acid and 29 grams (0.485 equivalents) of acetic acid at 90° C. The mixed acids were added dropwise. After only approximately one-half of the acid mixture had been added, the product gelled.

50 This example illustrates that a gel is obtained when the formic acid is pre-mixed with a  $C_2$  to  $C_5$  carboxylic acid.

#### EXAMPLE 4

55 To 100 grams (0.215 equivalents of  $CO_2$ ) of the calcium sulfonate-calcium carbonate product of Example 2 was added 2.5 grams (0.049 equivalents) of 90.5% formic acid dropwise at 90° C. Afterward, the reaction mixture was heated to 120° C. and 5.1 grams (0.097 equivalents) of 97.4% of acetic anhydride was added slowly above the surface dropwise. The reaction mixture was cooled to 90° C. and another 2.5-gram portion (0.049 equivalents) of formic acid was added in the same manner as before. After the acid additions were completed, the mixture was heated to 150° C. in a stream of nitrogen for one hour. The mixture was cooled to 120° C. and 5 grams of diatomaceous earth filter aid was added. The mixture was filtered through diatomaceous earth filter aid on a heated Buchner funnel. The resulting product was a liquid.

## Analysis of product:

|                                              |         |     |
|----------------------------------------------|---------|-----|
| Calcium                                      | percent | 4.9 |
| Carbon dioxide                               | do      | 1.8 |
| Formic acid <sup>1</sup>                     | do      | 2.8 |
| Acetic acid <sup>1</sup>                     | do      | 4.3 |
| Perchloric acid base No. (mg. KOH/g. sample) |         | 114 |

<sup>1</sup> As formate and acetate of calcium.

## EXAMPLE 5

To 150 grams (0.30 equivalents of CO<sub>2</sub>) of a calcium sulfonate-calcium carbonate product similar to that used in Example 2 was added 3.65 grams (0.072 equivalents) of 90.5% of formic acid at 85° C. dropwise. The reaction mixture was heated to 120° C. and 3.75 grams (0.072 equivalents) of 97.4% of acetic anhydride was added slowly above the surface dropwise. The reaction mixture was cooled to 90° C. again and the two steps were repeated using the same conditions and amounts of acids as used in the first two steps, so that a total of about 0.288 equivalents of the acids were obtained in the four acid additions. The mixture was heated to 150° C. in a nitrogen stream for one hour. The mixture was then cooled to 120° C., and 7.5 grams of diatomaceous earth filter aid was added. The product was filtered through diatomaceous earth filter aid on a heated Buchner funnel. The resulting product was a liquid.

## Analysis of Product:

|                                              |         |      |
|----------------------------------------------|---------|------|
| Calcium                                      | percent | 4.7  |
| Carbon dioxide                               | do      | 2.01 |
| Formic acid <sup>1</sup>                     | do      | 5.99 |
| Acetic acid <sup>1</sup>                     | do      | 4.5  |
| Perchloric acid base No. (mg. KOH/g. sample) |         | 115  |

<sup>1</sup> As formate and acetate of calcium.

## EXAMPLE 6

To two samples of 100 grams of the calcium sulfonate-calcium carbonate used in Example 2 were added acetic anhydride and acetic acid, respectively, in equivalent amounts. When approximately 1/2 the acid had been added, in each case the reaction mixture gelled.

## EXAMPLE 7

To 500 grams (2.18 equivalents of CO<sub>2</sub>) of an over-based calcium sulfonate-calcium carbonate product containing 11.2% Ca, 9.6% CO<sub>2</sub> and a 303 TBN in a 1 liter, 4-neck round bottom flask equipped with a mechanically driven glass paddle stirrer, thermometer, a subsurface dropping funnel, and a water receiver adapted for nitrogen sparging and a condenser was added 61.2 grams (1.2 equivalents) of 90% formic acid at 200° C. A stream of nitrogen was used. The formic acid was added in two portions over an hour period each. A thirty minute hold time was maintained during the additions. The reaction mixture was maintained at 200° C. for 1/2 hour and 61.6 grams (1.2 equivalents) of 99.5% acetic anhydride was added in two portions using the same conditions as with the formic acid addition. The mixture was heated at 200° C. for one hour, cooled to 150° C., and 25 grams of diatomaceous earth filter aid was added. The mixture was filtered through diatomaceous earth filter aid on a heated Buchner funnel. The product was a liquid.

## Analysis of Product:

|                                          |         |       |
|------------------------------------------|---------|-------|
| Calcium                                  | percent | 10.6  |
| Carbon dioxide                           | do      | 3.4   |
| Sulfur                                   | do      | 0.66  |
| Base No. (HClO <sub>4</sub> ) mg. KOH/g. |         | 284   |
| KV at 210° F.                            | cs      | 77.25 |

## EXAMPLE 8

Using the same conditions, equipment and amount of sulfonate complex as in Example 7, the amount of formic acid was 31 grams (0.6 equivalents) and the amount of

acetic anhydride was 93.5 grams (1.8 equivalents). The product was a liquid.

## Analysis of Product:

|                                          |         |       |
|------------------------------------------|---------|-------|
| Calcium                                  | percent | 10.6  |
| Carbon dioxide                           | do      | 3.8   |
| Sulfur                                   | do      | 0.6   |
| Base No. (HClO <sub>4</sub> ) mg. KOH/g. |         | 286   |
| KV at 210° F.                            | cs      | 241.6 |

## EXAMPLE 9

Using the same equipment, conditions and amount of sulfonate product as in Example 7, 24.8 grams (0.485 equivalents) of 90% formic acid and 99.5 grams (1.9 equivalents) of 97.8% acetic anhydride were used. The amount of formic acid is equivalent to about 20% of 2.18 equivalents of CO<sub>2</sub> with a 10% excess; the formic acid was added in one portion. The amount of acetic anhydride is equivalent to about 80% of 2.18 equivalents of CO<sub>2</sub> with a 10% excess; the acetic acid anhydride was added in three equal portions. The product was a liquid.

## Analysis of Product:

|                                          |         |       |
|------------------------------------------|---------|-------|
| Calcium                                  | percent | 10.1  |
| Carbon dioxide                           | do      | 3.6   |
| Sulfur                                   | do      | .76   |
| Base No. (HClO <sub>4</sub> ) mg. KOH/g. |         | 282   |
| KV at 210° F.                            | cs      | 159.0 |

## EXAMPLE 10

To 2500 grams (10.9 equivalents of CO<sub>2</sub>) of the sulfonate product of Example 7 were added 513 grams (about 9 equivalents) of 90% formic acid at 200° C. dropwise. The addition was made in 3 portions. The mixture was maintained at 200° C. and 57 grams (about 1 equivalent of 99.5% acetic anhydride) was added in 1 portion. At the end of the acid additions, the reaction product was treated as in Example 7. The product was a liquid.

## Analysis of Product:

|                                          |         |      |
|------------------------------------------|---------|------|
| Calcium                                  | percent | 10.3 |
| Carbon dioxide                           | do      | 2.5  |
| Sulfur                                   | do      | 0.69 |
| Base No. (HClO <sub>4</sub> ) mg. KOH/g. |         | 2.84 |

## EXAMPLE 11

Following the same procedure as in Example 7, 19 grams (0.372 equivalent) of 90% formic acid was added to the sulfonate product at 200° C., then 106.3 grams (2.04 equivalents) of acetic anhydride was to be added in three separate portions. The first addition took one hour. The reaction mixture became a solid gel during the second addition.

## Evaluation of products

The fluid products of this invention were evaluated in the panel coker test and in the water stability test.

Panel coker test.—This test is used to determine the tendency of lubricants to form solid decomposition products when in contact with high temperature surfaces; this tendency indicating the high temperature, oxidation stability of the oil formulation.

A sample of the lubricant is splashed onto a weighed and polished aluminum test panel. The test panel is heated and placed in a coking apparatus in such a position that the polished surface thereof is exposed to contact with oil thrown against it by means of a splasher immersed in the oil. The test panel is heated to a temperature of 600° F. and maintained at this temperature while the splasher is "on and off" operated for a period of 24 hours. The splasher operates 15 seconds out of every minute. After the test, the panel is removed, cooled, washed, dried, and reweighed. The difference in weight before and after the test is the amount of solid combustion deposits. Comparison with base stocks containing other formulations in-

dicates the relative oxidation stability at high temperatures of the formulation components presently being tested.

To a mixture of paraffinic solvent refined mineral oils of SAE 30 was added 13.6% by weight of the calcium sulfonate-calcium carbonate reactant of Example 7 (Composition A). To a second sample of the same base stocks were added 14.1% of the carboxylate product of Example 7 (Composition B). Each sample of oil was formulated to provide a 40 TBN oil. The following results were obtained:

| Composition: | Weight deposit, mg. |
|--------------|---------------------|
| A            | 540                 |
| B            | 196                 |

Water stability test.—In this test, an oil formulation is evaluated for ability of a formulated oil to separate from water as completely as possible so that no water remains in the oil phase. Often, the presence of oil additives, such as detergents have emulsifying tendencies in which case many such formulated oils perform poorly in this test.

The oil formulation to be tested is mixed vigorously with 5% by volume of distilled water for three minutes and then allowed to stand for 24 hours. The results are rated by visual means. A rating of very good is one in which the oil and water separate to give 95% and 5% of each phase. If some water remains in the oil phase but the separation is still 95% and 5% oil-in-water respectively, the rating is good.

To the same base stocks are used in the panel coker test, containing a minor amount of a commercial calcium additive, was added 29.1% of a formated product of the calcium sulfonate-calcium carbonate salt used in Example 7. Such products are described and claimed in copending application Ser. No. 282,548 (Composition C). To a second sample of a base blend was added 28.1% of the carboxylate product of Example 7 (Composition D). To a third base blend was added 28.0% of the product of Example 8, (Composition E). The following results were obtained:

| Composition | Percent oil-water phase                   | Rating     |
|-------------|-------------------------------------------|------------|
| C           | 95 trace emulsion, 5 emulsion precipitate | Good.      |
| D           | 95 clear oil, 5 emulsion precipitate      | Very good. |
| E           | do                                        | Do.        |

The mixed formate-C<sub>2</sub>-to-C<sub>5</sub> carboxylate products of this invention represent an improvement over the carbonate-sulfonate product in that it has improved high temperature stability properties. These products show an improvement even over the formated derivatives in the water stability test. The products of this invention may find utility in the lubrication of automobile engines and in the diesel engines, such as used in trucks, ships and railroads. These derivatives may be used in both mineral oils and synthetic oils, such as esters and polyolefin fluids and the like. The lubricant formulations containing the derivatives of this invention may also be used in greases in which conventional thickeners are employed. Other additives may also be employed along with these derivatives as indicated in the water stability test, including antioxidants, pour point depressants, and the like. Oil compositions containing a minor amount, from 0.05% to about 50% by weight of the additive, find suitable use in the lubricating field. The compounds of this invention may be also used in aqueous emulsions, such as used in metal working operations.

Although the preparation and utility of certain of the products and oil compositions containing them have been set forth in detail, the present invention is not in any way limited to these specific embodiments but suitable modifications can be made therefrom without departing from the scope of the invention.

Having described our invention, we claim:

1. An oil-soluble overbased metal sulfonate liquid product obtained by the process comprising reacting an

alkaline earth metal carbonate overbased alkaline earth metal sulfonate product, which possesses a metal content of at least 200% higher than that of the corresponding normal metal sulfonate salt, with formic acid and a C<sub>2</sub> to C<sub>5</sub> carboxylic acid at a temperature of from 50° to 225° C., wherein the mole ratio of formic to the said C<sub>2</sub> to C<sub>5</sub> carboxylic acid is in the range of from about 40:1 to about 1:4, wherein the total acid equivalents are sufficient to substantially completely convert the metal carbonate component to the corresponding metal formate-C<sub>2</sub> to C<sub>5</sub> carboxylate, and wherein the formic acid is reacted with the metal carboxylate prior to reaction with the C<sub>2</sub> to C<sub>5</sub> carboxylic acid.

2. The product of claim 1 wherein the mole ratio is from 10:1 to 1:3.

3. The product of claim 1 wherein the C<sub>2</sub> to C<sub>5</sub> carboxylic acid is acetic acid.

4. The product of claim 1 wherein the C<sub>2</sub> to C<sub>5</sub> carboxylic acid is acetic anhydride.

5. The product of claim 1 wherein the formic acid is reacted portionwise and the C<sub>2</sub> to C<sub>5</sub> carboxylic acid is reacted after the first portion of formic acid.

6. The product of claim 1 wherein the alkaline earth metal is calcium.

7. The product of claim 1 wherein the reactions are carried out in the presence of a diluent.

8. The product of claim 7 wherein the diluent is a lubricating oil.

9. A lubricating oil composition containing a minor amount sufficient to impart detergency thereto of the product of claim 1.

10. The method of preparing the product of claim 1 comprising (1) reacting an oil-soluble alkaline earth metal carbonate-overbased alkaline earth metal sulfonate product, which possesses a metal content of at least 200% higher than that of the corresponding normal metal sulfonate salt, with formic acid in a proportion less than that sufficient to convert the metal carbonate component to metal formate, and (2) reacting the reaction mixture of step (1) with a C<sub>2</sub> to C<sub>5</sub> carboxylic acid to substantially convert the remaining metal carbonate component to the metal C<sub>2</sub> to C<sub>5</sub> carboxylate, said reaction steps being carried out at a temperature of from 50° to 225° C., the mole ratio of formic acid to C<sub>2</sub> to C<sub>5</sub> carboxylic acid being from about 40:1 to about 1:4.

11. The method of claim 10 wherein step (1) and step (2) are insufficient to completely convert the metal carbonate component to the metal formate-C<sub>2</sub> to C<sub>5</sub> carboxylate, and step (2) is followed by step (3) reacting the remaining metal carbonate component from the reaction mixture of step (2) with formic acid.

12. The method of claim 11 wherein the amount of acids in steps (1), (2) and (3) is insufficient to completely convert the metal carbonate component and step (3) is followed by step (4) reacting the remaining metal carbonate component with a C<sub>2</sub> to C<sub>5</sub> acid.

13. The method of claim 10 wherein the C<sub>2</sub> to C<sub>5</sub> acid is acetic acid.

14. The method of claim 10 wherein the C<sub>2</sub> to C<sub>5</sub> acid is acetic anhydride.

15. The method of claim 10 wherein the alkaline earth metal is calcium.

16. A fuel composition comprising a normally liquid hydrocarbon fuel and a minor amount sufficient to impart detergency thereto of the product of claim 1.

#### References Cited

#### UNITED STATES PATENTS

3,242,079 3/1966 McMillen ----- 252-33

PATRICK P. GARVIN, Primary Examiner.